# EUROPEAN PATENT APPLICATION

(11) **EP 2 479 305 A1**
(43) Date of publication of application: **25.07.2012**
(21) Application number: 11151732.2
(22) Date of filing: 21.01.2011
(51) Int. Cl.: C22C 21/10, C22F 1/053

(54) **Method of manufacturing a structural automotive part made from a rolled Al-Zn alloy**

(71) Applicant: Aleris Aluminum Duffel BVBA, 2570 Duffel (BE)
(72) Inventor: Khosla, Sunil, 1941 BT, Beverwijk (NL)
(74) Representative: Müller Schupfner & Partner

(57) **Abstract**

The invention relates to method of manufacturing a formed aluminium alloy structural part or a body-in-white (BIW) part of a motor vehicle, the method comprising: (a) providing a rolled aluminium sheet product wherein the aluminium alloy is an AA7000 series aluminium alloy and having a gauge in a range of 0.5 to 4 mm and being subjected to a solution heat treatment and having been cooled, (b) forming the aluminium alloy sheet to obtain a three-dimensional formed part, (c) cooling of the formed part to a sub-zero temperature (T1) by immersing in a coolant, and allowing the formed part to reach equilibrium at said sub-zero temperature (T1), (d) heating of the formed part from the sub-zero temperature (T1) to a temperature T2 above 40°C, followed by cooling to ambient temperature, and (e) subjecting said motor vehicle component to a paint bake cycle.

## Description

### FIELD OF THE INVENTION

The invention relates to a method of manufacturing a formed aluminium alloy structural part or body-in-white (BIW) part of a motor vehicle, wherein the aluminium alloy is an AA7000-series alloy.

### BACKGROUND TO THE INVENTION

As will be appreciated herein below, except as otherwise indicated, aluminium alloy designations and temper designations refer to the Aluminum Association designations in Aluminum Standards and Data and the Registration Records, as published by the Aluminum Association in 2010.

For any description of alloy compositions or preferred alloy compositions, all references to percentages are by weight percent unless otherwise indicated.

Body-in-white consists of the structural components of the automobile, not including closures (e.g. door panels, hood panels, trunk lid panels).

In the production of motor vehicles in particular aluminium alloys the AA5xxx- and AA6xxx-series alloys like 5051, 5182, 5454, 5754, 6009, 6016, 6022, and 6111, have been used to produce automotive structural parts and body-in-white ("BIW") parts.

There is a demand for the use of aluminium alloys, in particular for formed structural and BIW parts, which are formable and having in particular increased strength after being subjected to a paint bake cycle. In addition, the properties normally required for such parts include a high formability for the forming operation (typically by means of stamping, deep drawing, or roll forming), high mechanical strength after paint baking so as to enabling down gauging thus minimising the weight of the part, good behaviour in the various assembly methods used in motor vehicle manufacturing such as spot welding, laser welding, laser brazing, clinching or riveting, and an acceptable cost for mass production.

### DESCRIPTION OF THE INVENTION

It is an object of the present invention to provide a method of manufacturing formed structural parts made from AA7000-series sheet alloy products.

It is another object of the invention to provide a method of manufacturing formed structural automotive parts made from AA7000-series sheet alloy products.

These and other objects and further advantages are met or exceeded by the present invention providing for a method of manufacturing a formed aluminium alloy structural part or a body-in-white (BIW) part of a motor vehicle, the method comprising the steps of:
a. providing a rolled aluminium sheet product wherein the aluminium alloy is an AA7000 series aluminium alloy and having a gauge in a range of about 0.5 mm to 4 mm, and preferably of about 0.7 to 3.5 mm, and being subjected to a heat treatment at a temperature placed in a phase field of the aluminium alloy where substantial strengthening is realised following a cooling operation, and including the often applied solution heat treatment ("SHT") followed by quenching,
b. forming the aluminium alloy sheet to obtain a three-dimensional formed part,
c. cooling of the formed part to a sub-zero temperature (T1) by immersing it in a coolant, and allowing the formed part to reach temperature equilibrium at the sub-zero temperature (T1),
d. heating of the formed part from the sub-zero temperature (T1) to an elevated temperature T2 of 20°C or more, followed by cooling to ambient temperature, and
e. subjecting the formed and heat-treated and cooled part to a paint bake cycle, and wherein said paint bake cycle results in a yield strength of at least 350 MPa in said AA7000-series alloy product.

In accordance with this invention it has been found that applying at least once a dedicated heat-treatment involving cooling or quenching to a sub-zero temperature followed by heating the formed part from the sub-zero temperature to ambient temperature (20°C) or more and followed by cooling to ambient temperature if it was heated to a higher temperature than ambient temperature, after forming of the sheet product but prior to the paint bake cycle significantly reduced the delayed fracture sensitivity of the formed aluminium part made from the AA7000-series aluminium alloy sheet product. It has been found that AA7000-series sheet alloys when formed for example by means of stamping into three-dimensional components can be sensitive to fracture cracking when at ambient temperature in an ambient atmosphere like in a press shop, thus in a commonly non-aggressive corrosive environment. This results in that the stamped components may show significant tendency to the formation of cracks not immediately during or upon the forming operation but with some delay of only after a few hours or even firstly after several days in an ambient environment. This phenomena is also referred to as sensitivity to delayed crack formation. However, when subjecting the formed component at least once to this dedicated heat-treatment the sensitivity to delayed fracture is significantly reduced and it can even be overcome.

The time between the forming operation and the cooling of the formed part to sub-zero temperatures is not too critical, but it is preferred to perform the cooling operation within 1 hour after the forming operation, and preferably within 30 minutes after forming, and more preferably if practical from a logistics point of view immediately after the forming operation.

In the method according to this invention the formed part is cooled to a sub-zero temperature T1 (°C), and wherein T1 is in the range of about minus 25°C to minus 200°C. And preferably of about minus 40°C to minus 200°C, thus for example to the temperature of liquid nitrogen (minus 196°C) or to the temperature of dry ice having a temperature of minus 78°C. While quenching or cooling to the sub-zero temperature (T1) was performed by cryogenic cooling using liquid nitrogen or dry ice and which are preferred, it should be understood that quenching may also include other types of cooling liquids (dry ice/ethanol, dry ice/acetone, liquid nitrogen/solvent, and the like) or gases.

Once quenched to the sub-zero temperature the formed part should be allowed to reach equilibrium at this temperature. Once equilibrium is attained, the formed part will be uniform in temperature.

Thereafter the sub-zero temperature cooled and formed part is rapidly heated to a temperature T2 of ambient temperature (about 20°C) or more. From a metallurgical perspective the upper limit for T2 is about 250°C, and more preferably about 200°C, and even more preferably about 120°C. Although the residential time at temperature T2 is short, any uncontrolled precipitation is to be avoided. Furthermore, a too high temperature may introduce undesired residual stresses into the formed part when cooling back to ambient temperature. A preferred lower-limit for T2 is about 40°C. For example T2 could be about 80°C or about 100°C.

This rapid heating from T1 to elevated temperature T2 can be achieved be submerging the formed part into a hot liquid of temperature T2, e.g. boiling water, or by using convection heating or steam (e.g. by transferring of the formed part to a steam chamber having for example nozzles spraying hot water steam onto the formed part, and whereby for a high heat transfer for example high velocity steam is being applied).

And once at the elevated temperature T2 the formed part should be allowed to cool to ambient temperature, for example using regular air cooling, for further processing into a motor vehicle component.

The rolled aluminium alloy sheet may be obtained by methods known in the art, and which include continuous casting or DC-casting of a rolling stock, homogenisation and/or preheating of the rolling stock, hot rolling and/or cold rolling to a final gauge typically in the range of about 0.5 to 4 mm. Depending on the alloy composition and the amount of cold work an intermediate anneal may be used before or during the cold rolling operation.

The heat treatment such as a SHT and quenching of the sheet product can be carried out as a continuous operation for example using a continuous annealing line, after which the sheet product is being coiled again. The coiled sheet product can then be transported to a press shop for further processing into a formed part.

As the SHT and quenched sheet product is in an instable condition due to the occurrence of a spontaneous natural ageing effect at ambient temperature (in the art also referred to a W-condition), preferably the time between the quenching operation and the forming operation is less than 2 weeks and more preferably less than 4 days.

In an alternative embodiment the sheet product following SHT and quenching is artificially aged at a temperature in a range of 50°C to 250°C. For example to an underaged T6 temper, e.g. T61, T64 or T65 according to EN515. In a preferred embodiment the sheet product is aged to an over-aged T7x temper, for example a T79 temper. An advantage of using an over-aged temper is that during the paint-bake cycle there is substantially no further over-ageing, resulting in that there is no significant loss of strength in the sheet product as a consequence of the paint-bake cycle.

In an alternative embodiment the cold rolled sheet product is subjected to a heat treatment at a temperature placed in a phase field of the aluminium alloy where substantial strengthening is realised following a cooling operation, in particular it can be SHT followed by quenching, near or in the press shop such that the dwell time between cooling and the forming operation is being reduced. Depending on the logistic arrangements it may still be produced as a coiled product or alternatively firstly uncoiled, then cut in a separate sheet product having smaller dimensions, the cut sheet product being heat treated individually or in a small batch, subsequently cooled and formed, preferably within 4 hours after cooling, into a three-dimensional formed part or component.

If desired it is also possible that the heat treated and cooled sheet receives a controlled amount of stretching, typically in a range of 0.5% to 4%, to increase the flatness of the sheet product prior to any subsequent forming operation. In an alternative route the sheet product is compressed, typically in a range of 1% to 5%, for example using a die operation.

Following the heat treatment and cooling and optional stretching or compression, the sheet product can be formed into a three-dimensional formed BIW part or other structural component configuration of a motor vehicle.

The forming operation can be any forming operation used to shape three-dimensional motor vehicle components, and includes in particular operations like stamping, deep drawing, pressing, press forming, and roll forming, either at ambient or at elevated temperature.

Before shaping, the sheet product may be coated with a lubricant, oil or dry lubricant, suitable for the forming operation, the assembly and the surface treatment of the structural part to be produced.

Following the forming operation and the dedicated heat-treatment in accordance with this invention the formed part is typically made part of an assembly of other metal components as is regular in the art for manufacturing vehicle components, and subjected to a paint bake operation to cure any paint or lacquer layer applied. During the paint bake cycle the formed AA7000-series alloy product achieves its desired final strength levels. The paint bake operation or paint bake cycle typically comprises one or more sequential short heat treatment in the range of 140°C to 200°C for a period of 10 to less than 40 minutes, and typically of less than 30 minutes. A typical paint bake cycle would comprise a first heat treatment of about 180°C@20 minutes, cooling to ambient temperature, then about 160°C@20 minutes and cooling to ambient temperature. In dependence of the OEM such a paint bake cycle may comprise of 2 to even up to 5 sequential steps and includes drying steps, but either way the cumulated time at elevated temperature (100°C to 200°C) of the aluminium alloy product is less than 120 minutes.

The method according to this invention can be applied to a wide range of AA7000-series alloys, in particular those that show a tendency to natural ageing. In a preferred embodiment the aluminium alloy is selected from the group of AA7021, AA7136, AA7075, AA7081, AA7085, AA7050, AA7055, and modifications thereof.

In another preferred embodiment, the AA7000-series alloy comprises, in wt.%,

| | |
|---|---|
| Zn | 5.5 to 8, preferably about 6 to 7.5, |
| Mg | 1.5 to 2.1 |
| Cu | 0 to 0.45 |
| Mn | 0 to 0.15, preferably 0 to 0.05, |
| Zr | 0.04 to 0.25% |
| Ti | 0 to 0.15 |
| Fe | 0 to 0.35 |
| Si | 0 to 0.25, |

other elements and unavoidable impurities, each maximum 0.05%, total 0.20%, balance aluminium.

In an embodiment the AA7000-series aluminium alloy sheet product has been provided with a metal clad layer applied on at least one side, wherein the metal clad layer material has an inner-surface and an outer-surface and wherein the inner-surface is facing the AA7000-series material.

The clad layer or clad layers are usually much thinner than the core sheet, and each clad layer constituting about 1% to 25% of the total composite sheet thickness. A clad layer more typically constitutes around about 1% to 14% of the total composite sheet thickness.

The clad layer material can be made from an AA3000, AA4000-, AA5000-, AA6000-, or a different AA7000-series aluminium alloy compared to the core alloy.

In an embodiment the clad layer material consists of an AA5000-series alloy having more than 3.8% of Mg. More preferably the clad layer material has more than 4.8% of Mg, and preferably less than 7%, and more preferably less than 5.9%. With the application of the clad layer in particular the characteristics for the pretreatment like phosphating, passivation or alternative processes used at OEM's are improved. Aluminium alloys of the AA5000-series are known to the automotive industry and having an AA5000-series alloy as outersurface results in that there are little or no adjustments required for the surface pretreatment of the composite structure compared to aluminium alloys already in use for automotive applications. Hence there are no problems with existing alloy systems. Another advantage of the composite structure is it can be used for making components having a high impact resistance or good crash performance. The application of an AA5000-series clad layer having a high Mg-content results in a favourable formation of less cracks at the surface as these alloys have a good bendability, while the defined AA7000-series core alloy provides the required high strength.

In an embodiment the clad layer material consists of an AA6000-series aluminium alloy to increase the overall corrosion performance of the formed part. Preferred alloys are AA6016 and AA6005-series alloys.

Due to this high yield strength after a paint bake cycle, good formability and low weight, the BIW part manufactured according to this invention is an ideal candidate to replace parts made from dual-phase steel such as steel grades dp600, dp800, and boron steels, leading to considerable weight saving opportunities in the motor vehicle.

In a further aspect of the invention it relates to an formed structural motor vehicle part or a BIW part of a motor vehicle, the part being made from an AA7000-series aluminium alloy having a gauge in the range of 0.5 to 4 mm, and preferably in the range of 0.7 to 3.5 mm, and wherein the part has been SHT, quenched, formed from sheet into a three-dimensional formed part, and after being formed subject to a heat-treatment by holding it at a sub-zero temperature of less than minus 25°C and the heated to a temperature of more than 40°C and cooled to ambient temperature to reduce the sensitivity to delayed cracking at ambient temperature. Thereafter the heat-treated formed part can be subjected to a paint bake cycle to provide a yield strength of at least 350 MPa, and more typically of at least 400 MPa.

In another aspect of the invention it relates to a motor vehicle incorporating a formed aluminium alloy BIW part in accordance with this invention.

In the following, the invention will be explained by the following non-limitative example.

### Example.

Aluminium alloy sheet of 1.2 mm gauge and having a composition of about 7.3% Zn, about 1.95% Mg, about 0.07% Cu, about 0.1% Zr, balance impurities and aluminium, had been produced using a regular processing route. The sheet had been resolutionised and quenched (so-called "fresh W-temper") and immediately drawn into a cup using the well-known Erichson drawn-cup-test at ambient temperature and ambient atmosphere. Within 24 hours at ambient temperature and ambient atmosphere the drawn cup showed a serious formation of a series of cracks in the cup as shown in Fig. 1.

In accordance with the invention drawn cups were within about 2 minutes after drawing quenched in liquid nitrogen and kept at this temperature for about 15 minutes and then reheated to 200°C by transferring the cups to a pre-heated furnace of 200°C and kept at this temperature for about 20-30 minutes and cooled by air cooling to ambient temperature. The cups that being subjected to this heat treatment did not shown any formation of delayed fracture irrespective of the time after completion the heat treatment; thus no crack formation after several months. Five days after this heat treatment several cups had been subjected to a simulated paint-bake cycle and all remained fully intact following this paint-bake cycle.

The delayed fracture in drawn cups occurred also in the same sheet material but having been solution heat-treated, quenched and over-aged to a T79 temper prior to the drawing at ambient temperature and ambient atmosphere. Also here the identical heat treatment of quenching to sub-zero temperature and reheating to 200°C in accordance with this invention resulted in the avoidance of crack formation in the drawn cups, and several of these heat treated and drawn cups after 5 days had been successfully subjected to a simulated paint-bake cycle without any crack formation.

It will be appreciated by those of ordinary skill in the art that the method can be embodied in other specific forms without departing from the spirit or essential character thereof. The presently disclosed embodiments are therefore considered in all respects to be illustrative and not restrictive.

## Claims

1. Method of manufacturing a formed aluminium alloy structural part or a body-in-white (BIW) part of a motor vehicle, the method comprising:
a. providing a rolled aluminium sheet product wherein the aluminium alloy is an AA7000 series aluminium alloy and having a gauge in a range of 0.5 to 4 mm and being subjected to a solution heat treatment and having been cooled,
b. forming the aluminium alloy sheet to obtain a three-dimensional formed part,
c. cooling of the formed part to a sub-zero temperature (T1) by immersing in a coolant, and allowing the formed part to reach equilibrium at the sub-zero temperature (T1),
d. heating of the formed part from the sub-zero temperature (T1) to a temperature T2 above 40°C, followed by cooling to ambient temperature, and
e. subjecting said motor vehicle component to a paint bake cycle.

2. Method according to claim 1, wherein the formed part during step c. is cooled to a sub-zero temperature of -25°C or less, and preferably to a sub-zero-temperature in the range of -40°C to -200°C.

3. Method according to claim 1 or 2, wherein the formed part during step d.) is heated from temperature T1 to temperature T2 and wherein T2 is 20°C or more, and preferably T2 is less than 250°C.

4. Method according to any one of claims 1 to 3, wherein the formed part after step d.) and prior to the paint bake cycle is being assembled with one or more other metal parts to form an assembly forming a motor vehicle component.

5. Method according to any one of claims 1 to 4, wherein for said formed part the accumulated time at elevated temperature during the paint bake cycle is less than 120 minutes.

6. Method according to any one of claims 1 to 5, wherein the rolled aluminium sheet product has a metal clad layer on at least one side.

7. Method according to any one of claims 1 to 6, wherein the aluminium sheet product has a chemical composition within AA7021, AA7136, AA7075, AA7081, AA7085, AA7050, or AA7055.

8. Method according to any one of claims 1 to 6, wherein the aluminium sheet product has a composition of, in wt.%:
| | |
|---|---|
| Zn | 5.5 to 8, preferably 6 to 7.5, |
| Mg | 1.5 to 2.1 |
| Cu | 0 to 0.45 |
| Mn | 0 to 0.15, preferably 0 to 0.05, |
| Zr | 0.04 to 0.25% |
| Ti | 0 to 0.15 |
| Fe | 0 to 0.35 |
| Si | 0 to 0.25, |
other elements and unavoidable impurities, each maximum 0.05%, total 0.20%, balance aluminium.

9. Motor vehicle incorporating a formed body aluminium BIW part obtained by the method according to any one of claims 1 to 8.
